# EUROPEAN PATENT SPECIFICATION

(11) **EP 2 986 772 B1**
(45) Date of publication and mention of the grant of the patent: **25.07.2018**
(21) Application number: 14727233.0
(22) Date of filing: 18.04.2014
(51) Int. Cl.: D06M 15/03, D06M 10/10, D01F 11/00, D02G 3/00, D06M 10/00, D06M 11/11, D06M 11/53, D06M 16/00

(54) **A PROCESS OF MAKING A YARN HAVING SUITABILITY FOR WEAVING**
VERFAHREN ZUR HERSTELLUNG EINES WEBBAREN GARNS
PROCÉDÉ POUR FABRIQUER UN FIL ADAPTÉ AU TISSAGE

(30) Priority: 18.04.2013 EP 13164379; 19.04.2013 IT MI20130649
(43) Date of publication of application: 24.02.2016
(73) Proprietor: Canepa, Elisabetta, 22020 San Fermo della Battaglia (IT)
(72) Inventor: Canepa, Elisabetta, 22020 San Fermo della Battaglia (IT)
(74) Representative: Simino, Massimo
(86) International application number: PCT/IB2014/060834
(87) International publication number: WO 2014/170876

(56) References cited:
- WO-A2-2004/078063
- JP-A- H0 241 473
- JP-A- H0 813 341
- JP-A- 2000 073 280
- JP-A- 2004 131 647
- US-A- 5 501 711
- US-A1- 2003 134 120
- HOONSIK SHIN ET AL: "Effect of Ultraviolet Irradiation on Fixation of Chitosan on Cotton and Poly(Ethylene Telephthalate) Fabrics.", SEN'I GAKKAISHI, vol. 54, no. 8, 1 January 1998 (1998-01-01), pages 400-406, XP055093810, ISSN: 0037-9875, DOI: 10.2115/fiber.54.8_400
- DATABASE WPI Week 201326 Thomson Scientific, London, GB; AN 2013-B19590 XP002718113, & CN 102 747 450 A (JIANGSU KAILI CARPET CO LTD) 24 October 2012 (2012-10-24)

## Description

The present invention relates to a process of making a yarn, preferably a thin yarn having suitability for weaving features, particularly a yarn having natural animal fibers, vegetable fibers, synthetic polymer fibers, man-made natural fibers, continuous filaments of animal origin and/or discontinuous filaments of animal origin, to be used in a pure state or blended together.

As used herein, the term weaving is generally used both for designating warp-and-weft weaving and knit-weaving.

The invention also relates to a yarn, preferably a thin yarn, made of natural animal fibers, vegetable fibers, synthetic polymer fibers and/or man-made natural fibers, continuous filaments of animal origin and/or discontinuous filaments of animal origin, to be used in a pure state or blended together, obtained with such process.

As used herein, for example:
- thin yarns are intended to cover yarns having a yarn count ranging from 40 to 200 Nm, and preferably a yarn count ranging from 65 to 200 Nm;
- animal fibers are intended to cover fleece or hair fibers (such as wool, alpaca, vicuna, cashmere and others);
- continuous filaments of animal origin are intended to cover filaments obtained by reeling from whole cocoons (such as silk);
- discontinuous filaments of animal origin are intended to cover filaments obtained by unravelling from defective cocoons (such as waste silk);
- vegetable fibers are intended to cover all the fibers obtained from plants, shrubs, inflorescences, roots, leaves (such as cotton, flax, hemp, jute, coir, ramie, bamboo, and others);
- synthetic polymer fibers are intended to cover, for example, polyamide, polyester, acrylic, polypropylene fibers, and others;
- man-made natural fibers are intended to cover, for example, rayon viscose, modal, acetate, cupro, tencel® and others.

These yarns of the above mentioned type are known to be difficult to spin and weave, due to their thinness which makes them prone to breaking during spinning or later weaving.

Furthermore, at present the following needs are strongly felt in the field of yarns and weaving:
- enhancing mechanical properties, such as abrasion resistance, of a thin yarn, and reducing mechanical friction between weft yarns and warp yarns, for trouble-free weaving;
- developing an environment-friendly and low-power-consumption process of making a yarn having improved suitability for weaving features;
- developing a process of making a yarn having improved features in terms of high resistance to pilling, felting and rubbing, as well as superior mechanical properties while maintaining the desired softness, volume, brightness and lightness features;
- developing a process of making a yarn having improved dye affinity, or improved affinity for the later finishing steps, such as printing.

Documents US 2003/134120 A1, JP 2000 073280 A and CN 102 747 450 A disclose the application of chitosan to fibers before spinning.

Documents JP H02 41473 A, JP 2004 131647 A, as well as Hoonsik Shin et al. "Effect of Ultraviolet Irradiation on Fixation of Chitosan on Cotton and Poly(Ethylene Telephthalate) Fabrics.", SEN'I GAKKAISHI, vol. 54, no. 8, 1998, pages 400-406, disclose the cross-linking of chitosan after it has been applied to yarns or fabrics. The present invention is based on the problem of conceiving and providing a process of making a yarn having suitability for weaving features, which fulfills the above mentioned needs.

This problem is solved by a process of making a yarn having suitability for weaving features as defined in claim 1.

According to the invention, before the step of spinning, the fibers and/or filaments undergo a step of application of a reinforcement product comprising a composition of chitosan and/or derivatives thereof, and a subsequent step of crosslinking of the chitosan and/or derivatives thereof of said reinforcement product applied to said fibers and/or to said filaments, such that a crosslinked reinforcement polymer permanently anchored to said fibers and/or to said filaments is obtained from said chitosan and/or derivatives thereof.

Chitosan is a natural polymer derived from chitin, which is a protein contained in the exoskeleton of crustaceans, and is a nature-renewable material, since it is obtained from food industry byproducts.

A reinforcement product based on chitosan and/or derivatives thereof, used as a sizing agent for the fibers and/or filaments has better sizing properties than other natural substances. For instance, the addition of 5 to 15% carboxymethyl chitosan concentrations in the sizing step has provided increases in toughness of cotton fabrics by up to 55%, with 3% reduction of elongation.

The core of the invention consists in overcoming a technical prejudice existing in the field of yarns and weaving: i.e. that the chitosan polymer may only be used to impart a temporary effect to the fibers and/or filaments of the yarns, which is designed to disappear after a first washing step or in other finishing steps.

Unlike prior art teachings, the present invention provides crosslinking of chitosan and/or derivatives thereof, to ensure permanent adhesion of chitosan to the fibers and/or filaments, such that the beneficial effects of chitosan may be maintained with time.

The advantage of the step of crosslinking of chitosan and/or derivatives thereof is that the fibers and/or filaments of the yarn are imparted a considerable physical-mechanical resistance, a long-lasting sanitization effect, resisting many repeated washes with hot and/or soapy water, as well as a considerable improvement in the affinity of the fibers and/or filaments.

In a further auxiliary aspect, the technique of crosslinking chitosan and/or its derivatives for application to the fibers and/or filaments of the yarn before weaving is used against the prejudice existing in the field of yarns and weaving, particularly for valuable yarns/fabrics such as cashmere or silk: i.e. that crosslinking of chitosan causes an undesired structural stiffening on the surface of the fibers and/or filaments of the yarns, which is unacceptable for valuable yarns/fabrics.

Conversely, according to a further auxiliary aspect of the present invention, the fibers and filaments of the treated yarns are coated with a thin layer of reinforcement product, which is first crosslinked and then, if needed, mostly removed in a partial and calibrated manner, the rest of the crosslinked chitosan and/or derivatives thereof applied to the fibers and/or filaments maintaining its beneficial effects, as mentioned above.

The process of making a yarn having suitability for weaving features, according to the invention comprises the steps of:
- providing natural animal fibers, vegetable fibers, synthetic polymer fibers and/or man-made natural fibers, continuous filaments of animal origin and/or discontinuous filaments of animal origin, to be used in a pure state or blended together;
- performing one or more processing operations on said fibers and/or said filaments for preparing them to spinning, selected from the group comprising: washing, drying, blending, cleaning, opening, reeling, unravelling, carding, combing, parallelization of fibers and/or filaments, web formation, stretching/thinning, rove formation and/or dyeing and
- spinning said fibers and/or said filaments once one or more of said processing operations have been performed on said fibers and/or said filaments for preparing them to spinning, to obtain a yarn.

Advantageously, the process is characterized in that it comprises:
- a step of applying a reinforcement product comprising a composition of chitosan and/or derivatives thereof to said fibers and/or to said filaments, said step of applying said reinforcement product comprising a composition of chitosan and/or derivatives thereof to said fibers and/or to said filaments being carried out before spinning said fibers and/or said filaments, and
- performing a subsequent step of crosslinking of the chitosan and/or derivatives thereof of said reinforcement product applied to said fibers and/or to said filaments, such that a crosslinked reinforcement polymer is obtained from said chitosan and/or derivatives thereof, which is permanently anchored to said fibers and/or to said filaments.

Preferably, said step of crosslinking of the chitosan and/or derivatives thereof of said reinforcement product applied to said fibers and/or to said filaments, is carried out before the step of spinning of said fibers and/or said filaments.

Alternatively, said step of crosslinking of the chitosan and/or derivatives thereof of said reinforcement product applied to said fibers and/or to said filaments, may be carried out after the step of spinning of said fibers and/or said filaments.

Preferably, in order to facilitate the subsequent step of crosslinking of the chitosan and/or derivatives thereof, after said step of application of a reinforcement product comprising a composition of chitosan and/or derivatives thereof to said fibers and/or to said filaments, a drying step is provided, for drying said fibers and/or said filaments as well as said reinforcement product, before crosslinking the chitosan and/or derivatives thereof of said reinforcement product applied to said fibers and/or to said filaments.

Preferably, said step of crosslinking of the chitosan and/or derivatives thereof of said reinforcement product applied to said fibers and/or to said filaments before the step of spinning the fibers, is carried out by a step of UV exposure of said chitosan and/or derivatives thereof.

Preferably, the process of the invention comprises a step of partial and calibrated removal of the crosslinked reinforcement polymer from said fibers and/or said filaments, which is carried out before the step of spinning of said fibers and/or said filaments.

Alternatively, said partial and calibrated removal of said crosslinked reinforcement polymer from said fibers and/or said filaments may be carried out after or at the same time as the spinning step.

Preferably, said step of partial and calibrated removal of said crosslinked reinforcement polymer from said fibers and/or said filaments is carried out by a hydrolyzing desizing step, and more preferably by immersion in a hydrolyzing desizing solution.

Such hydrolyzing desizing solution:
- provides enzymatic desizing or
- provides chemical desizing, using hydrolyzing acids.

Preferably, said partial and calibrated desizing step, which does not involve complete removal of the crosslinked polymer applied on the fibers, is at least partially carried out by mechanical desizing, whereby the fibers to be desized are physically acted upon by abrasion, rubbing, brushing and/or by treatments adapted to remove part of the crosslinked chitosan and/or chitosan-derived polymer from the fibers, such as by ultrasonic treatment.

Such mechanical abrasion and/or rubbing treatment for partial and calibrated removal of the crosslinked chitosan and/or chitosan-derived polymer may be carried out on the yarn during weaving, e.g. by sliding the yarn in contact with special rigid surfaces. These rigid surfaces may consist of the surfaces of the teeth of the weaving comb, eyelets through which the yarn is slid during weaving, surfaces of rollers contacted by the sliding yarn during the weaving step, bristles of a brush, and others.

These mechanical abrasion and/or rubbing treatments may be carried out on yarn fibers even after the weaving or knitting step, i.e. by directly acting upon the finished fabric or knit. In this case, these mechanical treatments are advantageously carried out by brushing the fabric or the knit.

According to an alternative embodiment, the partial and calibrated mechanical desizing step for removing the crosslinked chitosan and/or chitosan-derived polymer from the fibers may be carried out by ultrasonic treatment of such fibers. Conveniently this may take place, for example, with the fibers immersed in a liquid in which an ultrasound-emitting probe is introduced.

Advantageously, the ultrasonic treatment of the fibers may be carried out at the same time as a step of weaving or finishing during which the fibers are already immersed in a bath, for example during a fiber washing or a fiber dyeing step before weaving of the yarn or the fabric or knit.

The possibility of performing partial and calibrated mechanical desizing of the crosslinked polymer on the fibers does not exclude the possibility that such step may be carried out before or after, and in addition to a partial and calibrated chemical or enzymatic desizing step.

A partial and calibrated desizing step using ultrasounds may be carried out at the same time as a chemical or enzymatic desizing step, using the same bath, which will afford a synergy of effects between the different desizing steps.

Preferably, the above mentioned step of partial and calibrated removal of said crosslinked reinforcement polymer from said fibers and/or said filaments will leave said crosslinked chitosan-derived reinforcement polymer on said fibers and/or said filaments, in an amount of 0.1-9% w/w based on the dry weight of said fibers and/or said filaments after said crosslinking step.

The above mentioned step of applying a reinforcement product comprising a composition of chitosan and/or derivatives thereof to said fibers and/or to said filaments may be carried out using various methods, such as: foularding, spraying, dipping, aerosol, atomization and/or at least partial coating of the fibers and/or the filaments.

Preferably, the composition of chitosan and/or derivatives thereof is a solution comprising:
- chitosan, preferably of low molecular weight, more preferably of 150,000 Da, degree of deacetylation 75-85%; viscosity 20-200 cps at a concentration range of 0.5-10% w/v, preferably 0.8-3% w/v, more preferably 1% w/v;
- acid aqueous solution and
- radical photoinitiator.

Preferably, said acid aqueous solution comprises acetic acid at a concentration of 1.5-3.8% v/v, preferably at a concentration of 1.8-2.22% v/v, more preferably at a concentration of 2% v/v.

Such solution may be prepared through the steps of:
- dissolving the chitosan of low molecular weight in an acid aqueous solution of acetic acid,
- adding the photoinitiator in an amount of 1.4-4% w/w based on the dry weight of chitosan, preferably 1.8-2.2% w/w based on the dry weight of chitosan, more preferably 2% w/w based on the dry weight of chitosan, and
- stirring the solution, preferably by magnetic stirring.

If the above mentioned step of applying a reinforcement product comprising a composition of chitosan and/or derivatives thereof to said fibers and/or to said filaments is carried out by dipping the latter into a bath of said composition, there will be preferably a bath ratio ranging from 1-7 to 1-35, more preferably a bath ratio ranging from 1-10 to 1-30, most preferably a bath ratio ranging from 1-16 to 1-24.

According to different embodiments of the process of the invention:
- if the above mentioned processing steps for preparation to weaving comprise a washing step, then said step of applying a reinforcement product comprising a composition of chitosan and/or derivatives thereof to said fibers and/or to said filaments may be advantageously carried out during said washing step;
- if the above mentioned processing steps for preparation to weaving comprise a blending step in a blending chamber, then said step of applying a reinforcement product comprising a composition of chitosan and/or derivatives thereof to said fibers and/or to said filaments may be carried out in said blending chamber during said blending step;
- if the above mentioned processing steps for preparation to weaving comprise a carding step, then said step of applying a reinforcement product comprising a composition of chitosan and/or derivatives thereof to said fibers and/or to said filaments may be carried out on the carded fibers and/or filaments, preferably immediately after the carding step;
- if the above mentioned processing steps for preparation to weaving comprise a combing step, then said step of applying a reinforcement product comprising a composition of chitosan and/or derivatives thereof to said fibers and/or to said filaments may be carried out on the combed fibers and/or filaments, preferably immediately after the combing step;
- if the above mentioned processing steps for preparation to weaving comprise a step for preparation of a tuft, a top, a web, a ribbon and/or a roving, then said step of applying a reinforcement product comprising a composition of chitosan and/or derivatives thereof to said fibers and/or to said filaments may be carried out on said tuft, said top, said web, said ribbon or said roving, or
- if the above mentioned processing steps for preparation to weaving comprise a dyeing step, then said step of applying a reinforcement product comprising a composition of chitosan and/or derivatives thereof to said fibers and/or to said filaments may be carried out on said fibers and/or said filaments before said dyeing step.

A yarn made of natural animal fibers, vegetable fibers, synthetic polymer fibers and/or man-made natural fibers, continuous filaments of animal origin and/or discontinuous filaments of animal origin, to be used in a pure state or blended together, which may be obtained with a process according to the present invention, comprises a crosslinked reinforcement chitosan and/or chitosan-derived polymer, which is applied to said fibers and/or to said filaments.

Preferably, such yarn has a count ranging from 40 Nm to 200 Nm, preferably from 65 Nm to 200 Nm.

In the light of the above disclosure, the process of the invention as described above, and the yarn that can be obtained with such process, can fulfill the needs addressed herein.

The above disclosure is susceptible to a number of changes and variants within the inventive concept, as outlined by the annexed claims.

## Claims

1. **A process of making a yarn having suitability for weaving features**, comprising the steps of:
- providing natural animal fibers, vegetable fibers, synthetic polymer fibers and/or man-made natural fibers, continuous filaments of animal origin and/or discontinuous filaments of animal origin, to be used in a pure state or blended together;
- performing one or more processing operations on said fibers and/or said filaments for preparing them to spinning, selected from the group comprising: washing, drying, blending, cleaning, opening, reeling, carding, combing, parallelization, web formation, stretching/thinning, rover formation and/or dyeing and
- spinning said fibers and/or said filaments once one or more of said processing operations have been performed on said fibers and/or said filaments for preparing them to spinning, to obtain the yarn, **characterized in that it comprises:**
- a step of application of a reinforcement product comprising a composition of chitosan and/or derivatives thereof to said fibers and/or to said filaments, said step of applying said reinforcement product comprising a composition of chitosan and/or derivatives thereof to said fibers and/or to said filaments being carried out before the step of spinning of said fibers and/or said filaments, and
- performing a subsequent step of crosslinking of the chitosan and/or derivatives thereof of said reinforcement product applied to said fibers and/or to said filaments, such that a crosslinked reinforcement polymer permanently anchored to said fibers and/or to said filaments is obtained from said chitosan and/or derivatives thereof.

2. A process of making a yarn as claimed in claim 1 wherein, in order to facilitate the subsequent step of crosslinking of the chitosan and/or derivatives thereof of said reinforcement product applied to said fibers and/or to said filaments, after said step of application of a reinforcement product comprising a composition of chitosan and/or derivatives thereof to said fibers and/or to said filaments, a drying step is provided, for drying said fibers and/or said filaments and said reinforcement product comprising a composition of chitosan and/or derivatives thereof applied to said fibers and/or to said filaments, before carrying out said step of crosslinking of the chitosan and/or derivatives thereof of said reinforcement product applied to said fibers and/or to said filaments.

3. A process of making a yarn as claimed in any of claims 1 to 2, comprising a step of partial and calibrated removal of said crosslinked reinforcement polymer from said fibers and/or said filaments carried out before said step of spinning of said fibers and/or said filaments.

4. A process of making a yarn as claimed in claim 1 or 2, comprising a step of partial and calibrated removal of said crosslinked reinforcement polymer from said fibers and/or said filaments carried out after said step of spinning of said fibers and/or said filaments.

5. A process of making a yarn as claimed in claims 3 or 4, wherein said step of partial and calibrated removal of said crosslinked reinforcement polymer from said fibers and/or said filaments is carried out by a hydrolyzing desizing step.

6. A process of making a yarn as claimed in claim 5, wherein said hydrolyzing desizing solution:
- provides enzymatic desizing or
- provides chemical desizing, using hydrolyzing acids.

7. A process of making a yarn as claimed in any of claims 3 to 6, wherein said step of partial and calibrated removal of said crosslinked reinforcement polymer from said fibers and/or said filaments is carried out by a mechanical desizing step, with fibers being acted upon by abrasion, rubbing, brushing and/or by treatments adapted to remove part of the crosslinked chitosan and/or chitosan-derived polymer from the fibers.

8. A process as claimed as claimed in claim 7, wherein said mechanical desizing step on the fibers to be desized by abrasion and/or rubbing is carried out by sliding the yarn in contact with rigid surfaces.

9. A process as claimed in claim 8, wherein said rigid surfaces consist of the surfaces of the teeth of the weaving comb, eyelets through which the yarn is slid during weaving, surfaces of rollers contacted by the sliding yarn, fabric or knit, and/or by the bristles of a brush.

10. A process as claimed in any of claims 7 to 9, wherein said mechanical desizing step for physically acting upon the fibers to be desized by abrasion and/or rubbing is carried out on the yarn during the weaving step.

11. A process as claimed in any of claims 7 to 9, wherein said mechanical desizing step by abrasion and/or rubbing is carried out by brushing the fabric or knit, or by sliding the fabric or knit in contact with rigid surfaces.

12. A process as claimed in claim 7, wherein said partial and calibrated mechanical desizing step for removing the crosslinked chitosan and/or chitosan-derived polymer from the fibers is carried out by ultrasonic treatment of such fibers, preferably while said fibers are immersed in a bath.

13. A process as claimed in claim 12, wherein said ultrasonic treatment of the fibers is carried out at the same time as a step weaving or finishing processing step, during which the fibers are already immersed in a bath.

14. A process of making a yarn as claimed in any of claims 1 to 13, wherein said step of applying a reinforcement product comprising a composition of chitosan and/or derivatives thereof to said fibers and/or to said filaments is carried out using a solution comprising:
- chitosan, preferably of low molecular weight, more preferably of 150,000 Da, degree of deacetylation 75-85%; viscosity 20-200 cps at a concentration range of 0.5-10% w/v, preferably 0.8-3% w/v, more preferably 1% w/v.

15. A process of making a yarn as claimed in any of claims from 1 to 14, wherein said yarn has a count ranging from 40 Nm to 200 Nm, preferably from 65 Nm to 200 Nm.

## Patentansprüche

1. **Verfahren zur Herstellung eines Garns mit Verwebbarkeitseigenschaften,** umfassend folgende Schritte:
- Bereitstellen von natürlichen tierischen Fasern, pflanzlichen Fasern, synthetischen Polymerfasern und/oder künstlich hergestellten natürlichen Fasern, kontinuierliche Filamente tierischen Ursprung und/oder diskontinuierliche Filamente tierischen Ursprungs, die in reiner Form oder miteinander vermischt zu verwenden sind;
- Durchführen einer oder mehrerer Verarbeitungsvorgänge an den Fasern und/oder Filamente zur Vorbereitung für das Verspinnen, ausgewählt aus der Gruppe umfassen: Waschen, Trocknen, Vermischen, Reinigen, Öffnen, Wickeln, Kardieren, Kämmen, Parallelisieren, Bahn bilden, Dehnen/Ausdünnen, Vorgarnbildung und/oder Färben und
- Verspinnen der Fasern und/oder Filamente, nachdem einer oder mehrere der Verarbeitungsvorgänge an den Fasern und/oder Filamenten zur Vorbereitung des Verspinnens ausgeführt wurden, um das Garn zu erhalten,
**dadurch gekennzeichnet, dass es Folgendes umfasst:**
- einen Schritt des Aufbringens eines Verstärkungsprodukts, umfassend eine Zusammensetzung aus Chitosan und/oder Derivaten davon auf die Fasern und/oder Filamente, wobei der Schritt des Aufbringens des Verstärkungsprodukts, umfassend eine Zusammensetzung aus Chitosan und/oder Derivaten davon auf die Fasern und/oder Filamente ausgeführt wird, bevor der Schritt des Verspinnens der Fasern und/oder Filamente ausgeführt wird und
- Ausführen eines anschließenden Schrittes des Vernetzens des Chitosans und/oder der Derivate davon des auf die Fasern und/oder Filamente aufgebrachten Verstärkungsprodukts, sodass ein vernetztes Verstärkungspolymer, das dauerhaft auf den Fasern und/oder Filamenten verankert ist, aus dem Chitosan und/oder den Derivaten davon erhalten wird.

2. Verfahren zur Herstellung eines Garns nach Anspruch 1, wobei zur Erleichterung des anschließenden Schrittes des Vernetzens des Chitosans und/oder der Derivate davon des auf die Fasern und/oder Filamente aufgebrachten Verstärkungsprodukts nach dem Schritt des Aufbringens eines Verstärkungsprodukts umfassend eine Zusammensetzung aus Chitosan und/oder Derivaten davon auf die Fasern und/oder Filamente ein Trocknungsschritt vorgesehen ist, um die Fasern und/oder Filamente und das Verstärkungsprodukt, umfassend eine Zusammensetzung aus Chitosan und/oder Derivaten davon, das auf die Fasern und/oder Filamente aufgebracht wurde, zu trocknen, bevor der Schritt des Vernetzens des Chitosans und/oder der Derivate davon des auf die Fasern und/oder Filamente aufgebrachten Verstärkungsprodukts ausgeführt wird.

3. Verfahren zur Herstellung eines Garns nach einem der Ansprüche 1 bis 2, umfassend einen Schritt des teilweisen, kalibrierten Entfernens des vernetzten Verstärkungspolymers von den Fasern und/oder Filamenten, der vor dem Schritt des Verspinnens der Fasern und/oder Filamente ausgeführt wird.

4. Verfahren zur Herstellung eines Garns nach Anspruch 1 oder 2, umfassend einen Schritt des teilweisen, kalibrierten Entfernens des vernetzten Verstärkungspolymers von den Fasern und/oder Filamenten, der nach dem Schritt des Verspinnens der Fasern und/oder Filamente ausgeführt wird.

5. Verfahren zur Herstellung eines Garns nach Anspruch 3 oder 4, wobei der Schritt des teilweisen, kalibrierten Entfernens des vernetzten Verstärkungspolymers von den Fasern und/oder Filamenten durch einen hydrolisierenden Entschlichtungsschritt ausgeführt wird.

6. Verfahren zur Herstellung eines Garns nach Anspruch 5, wobei die hydrolisierende Entschlichtungslösung:
- eine enzymatischen Entschlichtung bereitstellt oder
- eine chemische Entschlichtung durch Verwendung von hydrolisierenden Säuren bereitstellt.

7. Verfahren zur Herstellung eines Garns nach einem der Ansprüche 3 bis 6, wobei der Schritt des teilweisen, kalibrierten Entfernens des vernetzten Verstärkungspolymers von den Fasern und/oder Filamenten durch einen mechanischen Entschlichtungsschritt ausgeführt wird, bei dem die Fasern durch Abrieb, Reiben, Bürsten und/oder Behandlungen beaufschlagt werden, um einen Teil des vernetzten Chitosans und/oder des von Chitosan abgeleiteten Polymers von den Fasern zu entfernen.

8. Verfahren nach Anspruch 7, wobei der mechanische Entschlichtungsschritt der zu entschlichtenden Fasern durch Abrieb und/oder Reiben beim Gleiten des Garns in Kontakt mit starren Flächen ausgeführt wird.

9. Verfahren nach Anspruch 8, wobei die starren Flächen aus den Flächen der Zähnen des Webkamms, Ösen, durch die das Garn beim Weben gleitet, Rollenflächen, die vom gleitenden Garn, Gewebe oder Gewirke berührt werden, und/oder den Borsten einer Bürste bestehen.

10. Verfahren nach einem der Ansprüche 7 bis 9, wobei der mechanische Entschlichtungsschritt zum physikalischen Beaufschlagen der zu entschlichtenden Fasern durch Abrieb und/oder Reiben während des Webschrittes auf das Garn ausgeführt wird.

11. Verfahren nach einem der Ansprüche 7 bis 9, wobei der mechanische Entschlichtungsschritt durch Abrieb und/oder Reiben durch Bürsten des Gewebes oder Gewirkes oder beim Gleiten des Gewebes oder Gewirkes im Kontakt mit starren Flächen ausgeführt wird.

12. Verfahren nach Anspruch 7, wobei der teilweise, kalibrierte mechanische Entschlichtungsschritt zum Entfernen des vernetzten Chitosans und/oder des von Chitosan abgeleiteten Polymers von den Fasern durch Ultraschallbehandlung derartiger Fasern ausgeführt wird, vorzugsweise, wenn die Fasern in ein Bad eingetaucht sind.

13. Verfahren nach Anspruch 12, wobei die Ultraschallbehandlung der Fasern gleichzeitig mit einem Web- oder Fertigbehandlungs-Bearbeitungsschritt ausgeführt wird, in dem die Fasern bereits in ein Bad eingetaucht sind.

14. Verfahren zur Herstellung eines Garns nach einem der Ansprüche 1 bis 13, wobei der Schritt des Aufbringens eines Verstärkungsprodukts, umfassend eine Zusammensetzung aus Chitosan und/oder Derivaten davon, auf die Fasern und/oder Filamente ausgeführt wird durch Verwenden einer Lösung, umfassend:
- Chitosan, vorzugsweise mit geringem Molekulargewicht, insbesondere mit 150.000 Da, einem Deacetylisierungsgrad von 75-85%; einer Viskosität von 20-200 cps in einem Konzentrationsbereich von 0,5-10% w/v, vorzugsweise 0,8-3% w/v, insbesondere 1% w/v.

15. Verfahren zur Herstellung eines Garns nach einem der Ansprüche von 1 bis 14, wobei das Garn eine Feinheit im Bereich von 40 Nm bis 200 Nm, vorzugsweise von 65 Nm bis 200 Nm aufweist.

## Revendications

1. **Procédé de fabrication d'un fil ayant des caractéristiques d'aptitude au tissage,** comprenant les étapes consistant à:
- fournir des fibres animales naturelles, des fibres végétales, des fibres synthétiques de polymère et/ou des fibres naturelles artificielles, des filaments continus d'origine animale et/ou des filaments discontinus d'origine animale, à utiliser à l'état pur ou mélangés ensemble;
- effectuer un ou plusieurs opérations de traitement sur lesdites fibres et/ou lesdits filaments pour les préparer à la filature, choisies dans le groupe comprenant: lavage, séchage, mélange, nettoyage, ouverture, dévidage, cardage, peignage, parallélisation, formation de nappe, étirage/amincissement, formation de mèches de banc et/ou teinture et
- faire tourner lesdites fibres et/ou lesdits filaments une fois que l'une ou plusieurs desdites opérations de traitement ont été réalisées sur lesdites fibres et/ou lesdits filaments pour les préparer à la filature, pour obtenir le fil,
**caractérisé en ce qu'il comprend:**
- une étape d'application d'un produit de renforcement comprenant une composition de chitosane et/ou de ses dérivés auxdites fibres et/ou auxdits filaments, ladite étape d'application dudit produit de renforcement comprenant une composition de chitosane et/ou de ses dérivés auxdites fibres et/ou auxdits filaments étant réalisée avant l'étape de filature desdites fibres et/ou desdits filaments, et
- la réalisation d'une étape ultérieure de réticulation du chitosane et/ou de ses dérivés dudit produit de renforcement appliqué auxdites fibres et/ou auxdits filaments, de sorte qu'un polymère de renforcement réticulé ancré en permanence auxdites fibres et/ou auxdits filaments est obtenu dudit chitosane et/ou ses dérivés.

2. Procédé de fabrication d'un fil selon la revendication 1, dans lequel, afin de faciliter l'étape suivante de réticulation du chitosane et/ou de ses dérivés dudit produit de renforcement appliqué auxdites fibres et/ou auxdits filaments, après ladite étape d'application d'un produit de renforcement comprenant une composition de chitosane et/ou de ses dérivés auxdites fibres et/ou auxdits filaments, une étape de séchage est prévue pour sécher lesdites fibres et/ou lesdits filaments et ledit produit de renforcement comprenant une composition de chitosane et/ou des dérivés de ceux-ci appliqués auxdites fibres et/ou auxdits filaments, avant d'effectuer ladite étape de réticulation du chitosane et/ou de ses dérivés dudit produit de renforcement appliqué aux dites fibres et/ou aux dits filaments.

3. Procédé de fabrication d'un fil selon l'une quelconque des revendications 1 à 2, comprenant une étape d'élimination partielle et calibrée dudit polymère de renforcement réticulé desdites fibres et/ou desdits filaments réalisés avant ladite étape de filature desdites fibres et/ou lesdits filaments.

4. Procédé de fabrication d'un fil selon la revendication 1 ou 2, comprenant une étape d'élimination partielle et calibrée dudit polymère de renforcement réticulé desdites fibres et/ou desdits filaments réalisée après ladite étape de filature desdites fibres et/ou lesdits filaments.

5. Procédé de fabrication d'un fil selon les revendications 3 ou 4, dans lequel ladite étape d'élimination partielle et calibrée dudit polymère de renforcement réticulé desdites fibres et/ou desdits filaments est effectuée par une étape de désencollage par hydrolyse.

6. Procédé de fabrication d'un fil selon la revendication 5, dans lequel ladite solution de désencollage par hydrolyse:
- fournit un désencollage enzymatique ou
- fournit un désencollage chimique, en utilisant des acides hydrolysants.

7. Procédé de fabrication d'un fil selon l'une quelconque des revendications 3 à 6, dans lequel ladite étape d'élimination partielle et calibrée dudit polymère de renforcement réticulé desdites fibres et/ou desdits filaments est réalisée par une étape de désencollage mécanique, les fibres étant traitées par abrasion, frottement, brossage et/ou par des traitements adaptés pour éliminer une partie du chitosane réticulé et/ou du polymère dérivé du chitosane des fibres.

8. Procédé selon la revendication 7, dans lequel ladite étape de désencollage mécanique sur les fibres à désencoller par abrasion e/o frottement est effectué en faisant glisser le fil en contact avec des surfaces rigides.

9. Procédé selon la revendication 8, dans lequel lesdites surfaces rigides sont constituées des surfaces des dents du peigne de tissage, oeillets à travers lesquels le fil est glissé pendant le tissage, surfaces des rouleaux en contact avec le fil coulissant, tissu ou tricot, et/ou des poils d'une brosse.

10. Procédé selon l'une quelconque des revendications 7 à 9, dans lequel ladite étape de désencollage mécanique pour agir physiquement sur les fibres devant être désencollées par abrasion et/ou frottement est effectuée sur le fil pendant l'étape de tissage.

11. Procédé selon l'une quelconque des revendications 7 à 9, dans lequel ladite étape de désencollage mécanique par abrasion et/ou frottement est effectuée en brossant le tissu ou le tricot, ou en faisant glisser le tissu ou le tricot en contact avec des surfaces rigides.

12. Procédé selon la revendication 7, dans lequel ladite étape de désencollage mécanique partielle et calibrée pour éliminer le chitosane réticulé et/ou le polymère dérivé de chitosane des fibres est effectuée par traitement ultrasonique de telles fibres, de préférence pendant que lesdites fibres sont immergées dans un bain.

13. Procédé selon la revendication 12, dans lequel ledit traitement par ultrasons des fibres est effectué en même temps qu'une étape de traitement de tissage ou de finissage, au cours de laquelle les fibres sont déjà immergées dans un bain.

14. Procédé de fabrication d'un fil selon l'une quelconque des revendications 1 à 13, dans lequel ladite étape d'application d'un produit de renforcement comprenant une composition de chitosane et/ou de ses dérivés auxdites fibres et/ou auxdits filaments est effectué en utilisant une solution comprenant:
- le chitosane, de préférence de faible poids moléculaire, plus préférablement de 150.000 Da, le degré de désacétylation de 75 à 85 %; viscosité 20-200 cps à une plage de concentration de 0,5 à 10 % en poids/volume, de préférence de 0,8 à 3% en poids/volume, plus préférablement de 1 % en poids/volume.

15. Procédé de fabrication d'un fil selon l'une quelconque des revendications 1 à 14, dans lequel ledit fil a une numération allant de 40 Nm à 200 Nm, de préférence de 65 Nm à 200 Nm.
